

2,890,135

**VACUUM METALIZING HIGH TENSILE STEEL PARTS**

Gordon W. Jenkins, Pasadena, Calif., assignor to Anadite, Inc., South Gate, Calif., a corporation of California

No Drawing. Application February 19, 1958  
Serial No. 716,046

4 Claims. (Cl. 117—107)

My invention relates to improvements in the protection of high tensile strength steel parts, such as those used in aircraft construction, and more particularly to the vacuum metalizing of such parts to provide a protective coating in such a manner as to completely eliminate hydrogen embrittlement of the steel parts.

The coating of steel parts used in aircraft construction with protective metals, more particularly with cadmium, has become a practical necessity in aircraft construction, especially for protecting and maintaining the life of such steel parts. Such coatings, as far as known, have been applied exclusively by electroplating the steel parts to be protected.

However, while electroplated cadmium coatings have provided protection, it has been found that the electrolytic deposition of cadmium causes hydrogen embrittlement of the steel, and this has become a very serious problem, especially with high strength steels with a 180K p.s.i. or higher. In the manufacture of steel aircraft parts, their dimensions are kept as low as possible because of the desirability of reducing the added weight. Therefore, it is extremely desirable, and in many cases essential, to use very high tensile strength steels for parts which are subjected to severe stresses, such as aircraft landing gear. Where these high tensile strength steel parts are electrolytically coated with cadmium, hydrogen embrittlement occurs, and there is a definite danger in their use.

This problem of hydrogen embrittlement of high tensile strength steels has been solved by depositing a protective metal coating on the high tensile strength steel parts suspended in a vacuum chamber in which the protective metal is vaporized and the resulting vapors condensed on the surfaces of the steel parts.

The primary object of the present invention is, therefore, to provide a method for producing high tensile steel parts, particularly for aircraft construction which are coated with a protective non-corrosive metal and are free of hydrogen embrittlement.

In the electrolytic plating of steel aircraft parts, as for example with cadmium, a system of specifications or standards have been developed and promulgated in order to control the quality of the protective coating. It has been found that the high tensile strength steel parts, produced in accordance with the present invention, meet the standards and specifications required for electrolytically coated parts and at the same time are entirely free of hydrogen embrittlement, so that their strength as structural and operative members is unimpaired.

The vacuum vaporization of metals for the coating of objects to produce decorations and for other purposes is well known, and in accordance with the invention, the improved method is carried out in a vacuum chamber of suitable size, evacuated in accordance with known practice, by suspending the high tensile strength steel parts in the vacuum chamber and vaporizing the coating metal, as for example cadmium beneath the parts, so that the vapors flow over the suspended parts and condense on them.

The steel parts to be processed according to the invention having a tensile strength of 180K p.s.i. and above are cleaned, if necessary, but without the use of cathodic cleaning, acid pickling or cleaning by any means involving release of hydrogen. Any scale, grease, oil or rust is removed and the parts are sand blasted by light grit blasting with 180 mesh or finer grit. The sand blasted parts are then immediately racked and placed in a vacuum chamber, and a vacuum of 0.5 micron is developed in the chamber by suitable pumping equipment. The protective metal to be vaporized is then heated in the chamber in a position below the steel parts. A sufficient coating, as for example, .0005 inch of the vaporized metal, is attained in from 15 to 35 minutes. When the parts are placed in the chamber at room temperature, the maximum temperature attained by the steel parts during the vacuum metalizing is approximately 175° F.

After completing the desired coating of the protective metal, the parts are removed from the vacuum chamber and are ready for use or for the application of the usual paint or organic coating, without baking or heat treatment. Where cadmium is used as the protective metal in the vacuum metalizing process, as is preferred, the parts removed from the chamber do not have a bright appearance but have a dull matte or satin finish of gray-white metallic luster. The vacuum metalized cadmium coatings were found to accept post processing chemical treatments and organic coatings conveniently used on electroplated parts in accordance with standard aircraft finishing systems.

Steel aircraft parts coated with cadmium by vacuum deposition have been found to meet all the requirements with respect to adhesion, corrosion resistance, and other requirements specified by Federal Specification QQ-P-416, for electroplated coatings. In a particular instance, low alloy steel parts heat treated to 260K p.s.i. (thousands of pounds per square inch) minimum ultimate tensile strength were coated with cadmium by vacuum vaporization and deposition to the extent of from .0003" to .0005" and found to be free of hydrogen embrittlement. The vacuum metalizing procedure produces no change in tensile strength of the parts.

Adhesion tests were performed on sheet steel test specimens 1" by 4" and approximately 0.04" thick which were coated with cadmium by vacuum vaporization and deposition. These specimens coated with from 0.0003" to .0005" of cadmium were bent through an angle of 180° on a diameter equal to the thickness of the sheet and then examined at 4X magnification for evidence of separation of the cadmium from the steel sheet. No separations were found in these tests. It was found that, even with successive coatings of cadmium applied in as many as five cycles, there was no evidence of separation and no evidence of contact between the successive coats when examined under the microscope. The vacuum coating procedure has been checked with respect to the evenness of the coating over irregularly-shaped parts. A bolt, for example, was coated in four cycles without changing its position in the rack in the vacuum chamber. The shank of the bolt was found to have a coating of .0014 inch and almost an equivalent thickness was deposited in the thread. Keyways, slots and surfaces at right angles to each other receive uniform coatings in one application and good coats are thrown into holes that would remain uncoated in electrolytic processing.

The effectiveness of the process of protecting steel parts having a tensile strength above 180K. p.s.i. against corrosion by applying vacuum metalized coatings thereto was demonstrated by testing cadmium coatings applied in this manner according to Specification QQ-P-416. In this test the parts were subjected to a salt spray exposure for 192 hours, according to the standard procedure.

There was no rusting of the surfaces of the parts, or even along the lines scribed through the coating. In a particular instance, a high heat treat steel fighter landing gear forging was vacuum coated with .0005" cadmium and then given the salt spray exposure test for 192 hours. There was no rusting or blistering of the coating. In general, it was found that vacuum metalized coatings stood up better in the salt spray corrosion test than the electroplated cadmium coatings.

The importance of the process in connection with the elimination of embrittlement in high tensile strength steels is shown in the following table giving the results of tensile tests on electrolytic cadmium coated specimens and vacuum metalized cadmium coated specimens. The table shows the reduction of area measurements in each instance, in accordance with standard hydrogen embrittlement test methods used for many years.

| Electroplated (60 a.s.f.—6 min.) |                            |                           | Vacuum metalized |                            |                           |
|----------------------------------|----------------------------|---------------------------|------------------|----------------------------|---------------------------|
| Specimen                         | Tensile Ultimate, K p.s.i. | Percent Reduction of Area | Specimen         | Tensile Ultimate, K p.s.i. | Percent Reduction of Area |
| 1-----                           | 281.8                      | 0                         | 1-----           | 272.2                      | 47.5                      |
| 2-----                           | 292.1                      | 0                         | 2-----           | 274.5                      | 48.2                      |
| 3-----                           | 274.4                      | 0                         | 3-----           | 279.7                      | 44.1                      |
| 4-----                           | 276.7                      | 0                         | 4-----           | 275.1                      | 45.2                      |
| 5-----                           | 281.7                      | 0                         | 5-----           | 280.9                      | 47.3                      |
| 6-----                           | 269.7                      | 0                         | 6-----           | 280.9                      | 46.8                      |

The test specimens reported on in the above table were 1" gauge length, 0.250" diameter 4340 low alloy steel, heat treated to 260K p.s.i. minimum ultimate tensile strength. The thickness of coating of all specimens was .0003" to .0005" and the tensile strength measurements were taken within four hours after the coatings were applied. The electrolytically coated specimens were tested without baking.

Known types of apparatus may be employed for carrying out the improved process and the metal to be vaporized and deposited on the high tensile strength parts may be vaporized either directly by resistance heated tungsten wires or their equivalent or by placing the metal in small crucibles heated by resistance heating elements, the crucibles preferably being distributed across and lengthwise of the vacuum chamber below the rack on which the steel parts are assembled for coating. The racks are preferably rotatable or movable, or located in such a way that all surfaces of the parts may be coated. In carrying out the process with cadmium, substantially pure cadmium was employed in the crucibles, and in tests made on the coated parts, it was found that the coating consisted almost exclusively of pure cadmium with only traces of impurities.

Some of the parts coated with cadmium may be mentioned as examples. A high tensile strength hex-headed bolt showed the following dimensions. The head before sand blast measured .7435", after sand blast .7422 and after cadmium coating .7426. The shank had a diameter of .4360 before sand blast, .4355 after sand blast and .4359" after cadmium coating. Another part, a 4340 steel fitting having a tensile strength of 260K p.s.i. and having flat, round tapering and other surfaces showed very similar dimension changes. For example, a shank part before sand blasting had a diameter of .4975", after sand blasting .4972, and after cadmium coating by vacuum metalizing .4975".

While the invention has been described and illustrated particularly in connection with the vacuum deposition of cadmium on high tensile strength steel parts, it is to be understood that other metals and combinations of metals may be vacuum vaporized and deposited on the high tensile strength steel parts to provide the desired protective non-corrosive metal coating. Some of these metals and alloys are; aluminum, tin, zinc, tin and cadmium, tin and

zinc, tin-cadmium-zinc. Other metals which may be used alone or in various combinations are magnesium, chromium, nickel, copper and silver. In certain instances, the steel part may be coated with one of these vaporizable metals and then subsequently coated with a different metal. For example, nickel or chromium may be applied over cadmium. However, since many aircraft structural parts are ultimately coated with organic coatings, the vaporized cadmium or its equivalent in a protective vaporizable coating metal may be employed as the basic adherent coating. Cadmium is particularly well suited for this purpose, since it is relatively inexpensive, light in weight and durable.

The process of the present invention not only provides an adherent, durable protective coating for high tensile strength steel parts, but the process of vacuum deposition of cadmium completely eliminates hydrogen embrittlement and provides such parts free from dangerous failure.

I claim:

1. The method of coating high tensile strength steel parts having tensile strengths in excess of 180K p.s.i., comprising enclosing the steel part to be coated in a vacuum zone, applying a vacuum in said zone of the order of 0.5 micron, vaporizing cadmium metal as a protective corrosion-resistant metal in said zone, condensing the resulting cadmium metal vapor directly on said steel part to provide a substantially uniform coating of from 0.0003" to 0.0005" on said part, and effecting the vaporization of the cadmium metal and the direct coating of the steel part in the vacuum zone under temperature and other conditions which leave the tensile strength of the cadmium coated steel part unchanged, thereby producing a high strength steel part with an adherent protective cadmium metal coating and which is free of hydrogen embrittlement.

2. The method of coating high tensile strength steel structural parts for aircraft having tensile strengths in excess of 180K p.s.i., comprising enclosing the steel part to be coated in a vacuum zone, applying a vacuum in said zone of the order of 0.5 micron, vaporizing substantially pure cadmium in said zone, condensing the resulting cadmium vapor directly on said steel part to provide an adherent cadmium metal coating of from 0.0003" to 0.0005" on said part, and effecting the vaporization of the cadmium metal and the direct coating of the steel part in the vacuum zone under temperature and other conditions which leave the tensile strength of the cadmium coated steel part unchanged, thereby producing a high strength steel part with a protective cadmium coating and which is free of hydrogen embrittlement.

3. The method of preventing hydrogen embrittlement of high tensile strength steel aircraft parts free of hydrogen embrittlement and having tensile strengths in excess of 180K p.s.i. and protecting such parts against corrosion, comprising enclosing the steel part free of hydrogen embrittlement in a vacuum zone, applying a vacuum in said zone of the order of 0.5 micron, vaporizing cadmium metal as a protective corrosion resistant metal in said zone, condensing the resulting cadmium metal vapor directly on said steel part to provide an adherent cadmium metal coating of from 0.003" to 0.0005" on said part, and effecting the vaporization of the cadmium and direct coating of the steel part in the vacuum zone under temperature and other conditions which leave the tensile strength and hydrogen embrittlement characteristics of the cadmium coated steel part unchanged, thereby producing an adherent high strength steel part with a protective metal coating and which is free of hydrogen embrittlement without reducing its tensile strength.

4. In the protection of high tensile strength steel aircraft parts against corrosion where such parts have tensile strengths in excess of 180K p.s.i. and are free from hydrogen embrittlement, the method comprising enclosing such

a steel part in a vacuum zone, applying a vacuum in said zone of the order of 0.5 micron, vaporizing cadmium metal as a protective corrosion resistant metal in said zone, condensing and depositing the resulting cadmium metal vapor directly on the surfaces of said steel part during a period of from 15 to 35 minutes to deposit on said surfaces an adherent coating of from 0.0003" to 0.0005", and heating said metal part in the vacuum zone by the condensation of the cadmium vapor thereon to a temperature not exceeding approximately

5

175° F., whereby said high tensile strength and hydrogen embrittlement characteristics of said steel part are unchanged.

## References Cited in the file of this patent

## UNITED STATES PATENTS

|           |                      |               |
|-----------|----------------------|---------------|
| 2,237,314 | Queneau et al. ----- | Apr. 8, 1941  |
| 2,274,444 | Freed -----          | Feb. 24, 1942 |
| 2,382,432 | McManus et al. ----- | Aug. 14, 1945 |
| 2,726,179 | Ortlieb et al. ----- | Dec. 6, 1955  |

UNITED STATES PATENT OFFICE  
CERTIFICATE OF CORRECTION

Patent No. 2,890,135

June 9, 1959

Gordon W. Jenkins

It is hereby certified that error appears in the printed specification of the above numbered patent requiring correction and that the said Letters Patent should read as corrected below.

Column 2, line 28, for "conveniently" read -- conventionally --;  
column 4, line 63, for "0.003" read -- 0.0003" --.

Signed and sealed this 13th day of October 1959.

(SEAL)  
Attest:

KARL H. AXLINE  
Attesting Officer

ROBERT C. WATSON  
Commissioner of Patents